

# UNITED STATES PATENT OFFICE.

FRED JOHNSTON, OF CALGARY, ALBERTA, CANADA, ASSIGNOR OF ONE-HALF TO  
ANDREW ORR, OF CALGARY, ALBERTA, CANADA.

## PROCESS OF TREATING MATCHES IN ORDER TO RENDER THEM IMMUNE TO THE ACTION OF MOISTURE.

1,301,448.

Specification of Letters Patent. Patented Apr. 22, 1919.

No Drawing.

Application filed March 4, 1918. Serial No. 220,394.

*To all whom it may concern:*

Be it known that I, FRED JOHNSTON, of the city of Calgary, in the Province of Alberta, Canada, farmer, have invented a certain new and useful Process of Treating Matches in Order to Render Them Immune to the Action of Moisture, of which the following is a specification.

To render matches immune to the action of moisture prepare a mixture of resin and beeswax in the proportions of two parts of resin to one part of beeswax, heat the mixture in a vessel until the boiling point is reached and mix thoroughly by agitation. Allow the mixture to cool down ten degrees Fahrenheit and dip the matches with the ignition head downward into the liquid until about one half of the stem of the match is immersed then remove the matches and on cooling a thin film of the mixture will be

found to have adhered to the match which film is impervious to moisture, hard but not friable, and at the same time will not interfere with the ignition or burning qualities of the matches. The time required for the mixture to set is very short as both ingredients are solids.

What I claim is:—

The process of waterproofing matches, which consists of dipping them head downward in a mixture composed of two parts by weight of resin, and one part by weight of beeswax, heated to a temperature a few degrees below boiling, thereby coating the igniting material and the stem portion, all substantially as described.

FRED JOHNSTON.

Witnesses:

WILFRID J. GRAY,  
S. M. GRAY.